

# UNITED STATES PATENT OFFICE.

CARL RÜMLER, OF SCHÖNEBERG, NEAR BERLIN, GERMANY.

## PROCESS OF TREATING ALUMINIUM ARTICLES FOR THE FORMATION OF GALVANIC METALLIC COATINGS.

992,600.

Specification of Letters Patent.

Patented May 16, 1911.

No Drawing.

Application filed October 6, 1910. Serial No. 555,681.

To all whom it may concern:

Be it known that I, CARL RÜMLER, merchant, a subject of the King of Prussia, residing at Schöneberg, near Berlin, Germany, have invented certain new and useful Improvements in an Improved Process of Treating Aluminium Articles for the Formation of Galvanic Metallic Coatings; and I do hereby declare the following to be a full, clear, and exact description of the invention, such as will enable others skilled in the art to which it appertains to make and use the same.

The present invention relates to an improved process of forming galvanic metallic coatings on aluminium and consists in preliminarily freeing the aluminium article to be treated from grease or the like, cleaning it and then providing it in a preliminary bath with a thin film-like coating upon which any desired metallic coating may be deposited in the usual electrolytic baths employed for ordinary metals.

The essential feature of the present invention may be said to consist in the fact that the film-like deposit, which forms the basis for the actual metallic coating to be subsequently deposited, consists of a metallic alloy.

It has been found that by employing a metallic alloy an extremely adherent coating is obtained upon which any other desired metal can be deposited directly. The most suitable metallic alloy for the deposit is brass obtained from a bath containing a suitable copper and zinc salt. A bath consisting of double cyanid of copper and zinc is specially suited for forming this deposit, an adequate quantity of sulfite being added to the bath in order to prevent oxidation of the cyanid. It is also advantageous to add to the bath a small quantity of a salt having an alkaline reaction such for example as potash or soda. This solution however deposits a brass very rich in zinc and a coating of this is less adherent than if the alloy is poorer in zinc. The precipitated alloy should preferably contain not less than 50% of copper. Now it has been found that in order to obtain a deposit containing a sufficient percentage of copper it is necessary to add a small quantity of an alkaline haloid such for example as chlorid of potassium or iodid of potassium.

Good results are obtained with a preliminary bath of the following composition: 1 liter of water, 40-60 gr. of double cyanid of copper, 15-30 gr. of double cyanid of zinc, 40-80 gr. of commercial sodium sulfite, 10-25 gr. potash, 2-10 gr. of chlorid of potassium. For the double cyanids it is advantageous to employ the respective metallic salts with cyanid of potassium solution until the cyanid deposit formed is dissolved.

The anodes may be of brass or of copper and zinc anodes, or only copper anodes can be used, in which latter case, however, it is frequently necessary to regenerate the bath and replenish the double zinc cyanid. If the brass is to adhere well, in the first place it is essential to maintain a suitable voltage. The voltage depends upon the halogen ion employed. It must be highest when chlorid is present, say approximately 1.8 volts; bromid requires approximately 1.7 volts; iodid approximately 1.6 volts. It is advisable to have a current strength of from 2 to 3.6 amperes per square decimeter. The period for the formation of the thin film-like coating of metallic alloy on the aluminium may amount to from  $\frac{1}{2}$  a minute to 2 minutes. Preferably the article is only exposed to the current in the electrolyte for a period of substantially one minute.

Having now particularly described and ascertained the nature of my said invention and in what manner the same is to be performed, I declare that what I claim is:

1. A process for conditioning aluminum articles for the deposition of metallic coatings by electrolytic baths which consists in treating the article electrolytically in a bath comprising an aqueous solution of two or more metallic double cyanids, and a sulfite to prevent oxidation; as set forth.

2. A process for conditioning aluminum articles for the deposition of metallic coatings by electrolytic baths which consists in treating the article electrolytically in a bath comprising an aqueous solution of two or more metallic double cyanids, and a sulfite to prevent oxidation; by a current of from 1.6 to 1.8 volts, and a current strength of from 2 to 3.6 amperes per square decimeter; as set forth.

3. A process for conditioning aluminum articles for the deposition of metallic coat-

ings by electrolytic baths which consists in  
treating the article electrolytically in a bath  
containing double cyanid of copper, double  
cyanid of zinc, an alkaline sulfite, and an  
addition of an alkaline halogen, and of a  
salt producing an alkaline reaction such as  
potash or soda.

In testimony whereof, I affix my signature,  
in presence of two witnesses.

CARL RÜMPLER.

Witnesses:

ANTON PELSCHING,  
AUGUST FUGGER.